

May 2, 1933.

G. D. EVANS

1,906,557

FURNACE LINING

Original Filed March 14, 1928

FIG. 1.



FIG. 2.



FIG. 3.



Inventor  
George David Evans  
By his Attorney Albert M. Austin

## UNITED STATES PATENT OFFICE

GEORGE DAVID EVANS, OF BALTIMORE, MARYLAND, ASSIGNOR TO AMERICAN SMCET-  
ING AND REFINING COMPANY, OF NEW YORK, N. Y., A CORPORATION OF NEW  
JERSEY

## FURNACE LINING

Original application filed March 14, 1928, Serial No. 261,497. Divided and this application filed May 3,  
1930. Serial No. 449,464.

This invention relates to furnaces, and more particularly to furnace linings and a method of forming the same.

This application is a division of my co-pending application Serial No. 261,497, filed March 14, 1928, for Furnace lining.

This invention may be applied specifically to refining furnaces; for example, furnaces used in the refining of copper. Such furnaces 10 are commonly constructed with their inner walls of magnesite brick, which becomes worn during use as the result of the chemical action of the charge and of the mechanical forces resulting from the great temperature 15 range to which a furnace of this type is subjected. The invention provides a lining which may be applied to the face of the magnesite brick and will serve as a protection therefor, both against the chemical action of 20 the charge and against the intense heat of the interior of the furnace.

In accordance with the present invention, a coating of protective materials is applied to the face of the magnesite brick and caused 25 to be impregnated therein. This coating is gradually applied while the charge is being withdrawn from the furnace and while parts of the charge still adhere to the walls.

The invention also consists in certain new 30 and original features of construction and combinations of parts hereinafter set forth and claimed.

Although the novel features which are believed to be characteristic of this invention 35 will be particularly pointed out in the claims appended hereto, the invention itself, as to its objects and advantages, the mode of its operation and the manner of its organization may be better understood by referring to the 40 following description taken in connection with the accompanying drawing forming a part thereof, in which

Fig. 1 is a sectional view of a conventional type of furnace, showing the lining applied thereto in accordance with the present invention;

Fig. 2 is an enlarged detail view showing the lining and illustrating the bonding action between the lining and the wall; and

Fig. 3 is an enlarged detail view showing

the lining built up to a substantial thickness.

Like reference characters denote like parts in the several figures of the drawing.

In the following description and in the 55 claims parts will be identified by specific names for convenience, but they are intended to be as generic in their application to similar parts as the art will permit.

Referring to the drawing more in detail, 60 the invention is shown as applied to a furnace comprising an arch 1 and a pair of side walls 2, which may be formed of any suitable material, as, for example—silica, or magnesite brick. Suitable doors, 3 are provided through which the furnace may be charged, and the working conditions thereof controlled. Base 4 may be formed of any suitable material, such as brick or burned-in 65 quartz. 70

In the operation of a furnace of this type, in the refining of copper, a bath of molten copper is maintained at an elevation slightly below the bottom of doors 3 until the desired 75 metallurgical reactions have taken place. The charge is then tapped for subsequent treatment and the operation repeated with a fresh charge.

It has been found that in furnaces operated as above the molten copper adheres to 80 the walls and enters into the bricks themselves, which become impregnated to a substantial depth. The copper becomes oxidized, due to the strongly oxidizing conditions maintained in the furnace, and forms tenorite and cuprite. 85

The present invention takes advantage of the above mentioned copper coating and utilizes the same for forming a protective covering over the furnace walls. This is accomplished by forcing finely divided silica against the furnace walls while the charge is being withdrawn. The silica adheres to the film of molten copper and becomes firmly 90 embedded therein, while the heat of the furnace changes substantial amounts of the silica to tridymite, in which form it is stable between the temperatures of 870° and 1470° C. 95

The silica is sprayed, or otherwise thrown upon the walls just above the molten bath as 100

the charge is withdrawn until substantially the entire surface of the wall has been covered by the protective coating. The operation is repeated for subsequent charges and the coating 5 built up to the desired thickness due to the bonding action of the molten copper. A homogeneous mass of the composition above mentioned is obtained, which may be made to cover the entire inner wall 10 of the furnace and prevent the magnesite brick from becoming worn. It has been found in practice that the life of a brick when used in a furnace wall, as above mentioned, is materially increased, thereby increasing the 15 total time during which a furnace may be operated and decreasing the maintenance charge.

Although applicant is not aware of the exact nature of the changes undergone by 20 the various elements in carrying on this process, it is believed to take place in two stages, namely the silicious material is firmly bonded to the magnesite brick and enters into the interior thereof, while successive layers or 25 accumulations of this material are bonded upon the previous layers. This is thought to be accomplished by an assimilation of silica in the copper oxide with which the magnesite brick or the silica material is impregnated. 30 Analysis of the furnace lining has revealed, however, that definite quantities of cuprite, tenorite, tridymite and quartz are present. The amount of metallic copper remaining is 35 comparatively small, since under furnace conditions the above mentioned oxides have been formed. Because of the high temperature the quartz grains have been highly fractured and have been largely converted into tridymite.

40 It is obvious that a lining formed as above provides a strong protective coating for the furnace walls in the form of a single uniform mass. A copper refining furnace having a magnesite brick lining has been described for 45 purposes of illustration. It is to be understood, however, that the invention is not limited thereto but may be applied to other furnaces and to other lining materials.

50 While certain novel features of the invention have been shown and described and are pointed out in the annexed claims, it will be understood that various omissions, substitutions and changes may be made by those skilled in the art without departing from 55 the spirit of the invention.

What is claimed is:

1. The method of forming a furnace lining which comprises impregnating the furnace walls with molten copper, subjecting 60 the interior of the furnace to oxidizing conditions whereby said copper is partially converted to copper oxides, adding finely divided silica to the molten copper and copper oxides whereby the silica becomes bonded in 65 a matrix of said oxides and repeating said

operation until a coating of substantial thickness has been built up.

2. In lining furnaces the improvement that comprises establishing a bath of molten copper within the furnace to be lined, tapping the molten copper from said furnace whereby a layer of copper adheres to the furnace walls and applying finely divided silica to said layer of copper while same is in a molten condition whereby a protective lining is formed. 70

3. The method of operating a furnace in the refining of copper, which comprises forming a bath of molten copper within said furnace, gradually withdrawing the bath therefrom, whereby a film of copper remains on the furnace walls, and forcing against said film while still in a molten condition a quantity of finely divided silica, whereby said silica becomes firmly embedded therein 80 and forms a protective coating for said walls. 85

4. The improved method of lining a metallurgical furnace having magnesite brick walls which comprises applying silica to 90 said walls in the presence of molten copper and copper oxides whereby a protective lining is formed on said magnesite brick.

In testimony whereof I have hereunto set my hand and seal. 95

GEORGE DAVID EVANS.

100

105

110

115

120

125

130